

## UNITED STATES PATENT OFFICE.

HUGH S. COOPER, OF CLEVELAND, OHIO, ASSIGNOR TO KEMET LABORATORIES COMPANY, INC., A CORPORATION OF NEW YORK.

### ALLOY.

No Drawing.

Application filed February 11, 1925. Serial No. 8,520.

The present invention relates to an alloy for use in high-speed cutting tools and the like which is similar in physical properties and structural characteristics to those disclosed in my U. S. Patent No. 1,221,769.

My new alloy contains as essential components nickel or cobalt in preponderating proportion, substantial amounts of tungsten and titanium, and minor amounts of aluminum and silicon. Molybdenum or uranium may be present, replacing part or all of the tungsten.

An alloy possessing hardness and good cutting qualities has been prepared with the following composition: tungsten, 6.80%; titanium, 8.98%; aluminum, 7.87%; silicon, 4.75%; nickel, balance, except for carbon and a small undetermined amount of iron present as an impurity. However, my invention is not limited to this precise composition as alloys possessing good cutting qualities may be prepared within the range set forth in the following table: tungsten, 1% to 12%; titanium, 1% to 12%; aluminum, 4% to 10%; silicon, 2% to 6%; nickel, balance, except for carbon which may vary from 0.10% to 1.50%, the preferred carbon content being 0.50%.

It is possible to produce the alloy by various methods. One method consists in melting tungsten-, titanium-, aluminum-, silicon-, and nickel-containing materials in a graphite crucible in any suitable type of furnace and then casting in a carbon mold. No heat treatment of the alloy is required in order to render it suitable as a cutting tool.

I claim:

1. An alloy containing a preponderating amount of a metal having the properties of nickel and cobalt; from 1% to 12% each of tungsten and titanium; from 4% to 10% of aluminum; and from 2% to 6% of silicon.

2. An alloy containing from 4 to 10% aluminium, 2 to 6% silicon, 1 to 12% tungsten, 1 to 12% titanium, the balance being principally nickel.

3. A cutting tool composed of an alloy containing from 4 to 10% aluminum, 2 to 6% silicon, 1 to 12% each of tungsten and titanium, the balance being principally nickel.

In testimony whereof, I affix my signature.

HUGH S. COOPER.